

Dec. 27, 1960

E. R. BREINING

2,966,427

GAS PLATING OF ALLOYS

Filed Nov. 7, 1958



INVENTOR.  
ELMER ROBERT BREINING

BY

*Toulmin & Toulmin*  
ATTORNEYS

# United States Patent Office

2,966,427

Patented Dec. 27, 1960

1

2,966,427

## GAS PLATING OF ALLOYS

Elmer Robert Breining, Dayton, Ohio, assignor, by mesne assignments, to Union Carbide Corporation, New York, N.Y., a corporation of New York

Filed Nov. 7, 1958, Ser. No. 772,519

11 Claims. (Cl. 117—106)

This invention relates to the formation of alloys and particularly to phosphorous containing alloys such as those of nickel and iron.

Nickel-phosphorous alloys and to a lesser extent iron-phosphorous alloys find utility in a variety of applications. For example, nickel containing  $Ni_3P$  is relatively easily soldered, below 750° F. has good hardness characteristics and may be chrome plated for decorative applications. Such alloys are useful for example in electrical connectors, aircraft parts and the like. Further, bonding to other metals such as stainless steel, aluminum, nickel, copper and magnesium is advantageously achieved.

It is a primary object of this invention to describe a novel method for the attainment of alloys containing a base metal and a combination of the base metal with phosphorous.

Another object of the invention is to describe a process for the production of phosphorous containing alloys having a high degree of purity.

A particular object of the invention is the provision of an alloy of nickel phosphorous or iron phosphorous achieved by deposition of the components from the gaseous state.

In the practice of the invention a volatile phosphorous component such as phosphine, phosphorous itself, or organic phosphorous compounds, such as the alkyl and aryl, is volatilized. Nickel carbonyl or other volatilizable, heat decomposable metal bearing compound is present to a reaction chamber with the volatilized phosphorous component. The reaction chamber contains an object upon which a film of the alloy is to be deposited and this object is suitably heated to effect decomposition of the gases.

The decomposition of the metal bearing gas in the case of nickel carbonyl provides nickel as the base metal; iron pentacarbonyl provides iron as the base metal.

Simultaneous co-deposition of the phosphorous component and the metal bearing gas provide on the heated object the alloy. Specific characteristics in the alloy are attained by combining more or less of the phosphorous component with the metal bearing component in the gaseous state. In the case of nickel carbonyl and tri-methyl phosphine the alloy desired contains nickel metal and  $Ni_3P$ . The content of  $Ni_3P$  controls the ultimate properties of the product and the  $Ni_3P$  is dispersed throughout the nickel phase.

Tri-methyl phosphine is a preferred source of the phosphorous as it has a boiling point close to that of nickel carbonyl and volatilization is more readily controllable than with phosphine, for example, where high reaction temperatures are required due to the stability of the phosphine.

Tri-ethyl phosphine which has a higher boiling point is more suitable when iron pentacarbonyl is employed. However, methyl di-ethyl phosphine, methyl ethyl propyl phosphine and others though somewhat more expensive presently, will serve the purpose.

2

The alloy deposition rate is a function of the flow rate of the phosphorous and base metal components, the temperature of the article being plated and to some extent the area of the object and the size of the plating chamber.

5 Deposition rate of 2 to 10 mils per hour are practicable while thickness may be from 0.1 mil to 10 mils or more. The flow sheet illustrates the essential steps of the process.

As will be noted from the flow sheet a liquid phosphorous containing component and a liquid metal bearing component are passed to a flash vaporizer and then to a reaction chamber wherein the heated object is contained. If desired a carrier gas, such as nitrogen, argon or carbon dioxide may be utilized to aid the flow of the vaporized materials to the reaction chamber. Within the reaction chamber the mixed gases contact the heated object and deposit thereon, forming a coating of the alloy.

As a specific example, liquid tri-methyl phosphine and nickel carbonyl are metered separately to a common 20 flash vaporizer along with the flow of carrier gas and are then transported to the plating chamber. Specific conditions are:

|                                            |               |          |
|--------------------------------------------|---------------|----------|
| Sample area                                | square inches | 10       |
| Substrate                                  | Steel         |          |
| 25 Tri-methyl phosphine, liquid            | cc./min       | 3.5-10   |
| Nickel carbonyl, liquid                    | cc./min       | 2-4      |
| Inert gas, $CO_2$                          | cc./min       | 400-1000 |
| Vaporizer temperature                      | ° F.          | 112-170  |
| 30 Specimen temperature                    | ° F.          | 350-700  |
| Phosphorous content of deposit ( $Ni_3P$ ) | percent       | 1-10     |
| Nickel content of deposit                  | do            | 99-90    |

As exemplary of the use of iron pentacarbonyl for the formation of an alloy containing iron and iron phosphorous the following data are applicable:

|                                                           |               |         |
|-----------------------------------------------------------|---------------|---------|
| Sample area                                               | square inches | 10      |
| Substrate                                                 | Steel         |         |
| 40 Tri-ethyl phosphine, liquid                            | cc./min       | 2.5-10  |
| Iron pentacarbonyl, liquid                                | cc./min       | 2-4     |
| (Optional) carbon dioxide                                 | cc./min       | 400-850 |
| Vaporizer temperature                                     | ° F.          | 260-285 |
| Substrate temperature                                     | ° F.          | 400-800 |
| 45 Phosphorous content of deposit ( $Fe_3P$ and $Fe_2P$ ) | percent       | 2-14    |
| in an iron matrix                                         | do            | 98-86   |

Copper may be substituted for the steel substrate in the foregoing samples.

50 The phosphines, particularly the alkyl phosphines and the aryl phosphines, are available and many have characteristics which would render them suitable, such as butyl phosphine and di-butyl phosphine, as well as cyclohexyl phosphine and phenyl phosphine, also alkyl halide phosphorous compounds have properties indicating utility 55 in the process.

It will be understood that this invention is susceptible to modification in order to adapt it to different usages and conditions and accordingly, it is desired to comprehend such modifications within this invention as may fall 60 within the scope of the appended claims.

What is claimed is:

1. The process of alloy formation which comprises combining in the vapor state a volume of a heat decomposable phosphorous component and a volume of a heat decomposable metal bearing gas, and contacting an object heated to the decomposition temperature of the combined vapors to effect deposition of a phosphorous containing alloy on the object.

70 2. The process of alloy formation which comprises combining in the vapor state a volume of a heat decomposable phosphorous component and a volume of gaseous

nickel carbonyl, and contacting an object heated to the decomposition temperature of the combined vapors to effect deposition of a phosphorous-nickel alloy on the object.

3. The process of alloy formation which comprises combining in the vapor state a volume of a heat decomposable phosphorous component and a volume iron pentacarbonyl, and contacting an object heated to the decomposition temperature of the combined vapors to effect deposition of a phosphorous-iron alloy on the object.

4. The process of alloy formation which comprises the steps of combining in the vapor state a volume of tri-methyl phosphine and a volume of gaseous nickel carbonyl, and contacting an object heated to the decomposition temperatures of the vapors to effect deposition of a phosphorous-nickel alloy on the object.

5. The process of alloy formation which comprises the steps of combining in the vapor state a volume of triethyl phosphine and a volume of gaseous iron pentacarbonyl, and contacting an object heated to the decomposition temperature of the combined vapors to effect deposition of a phosphorous-iron alloy on the object.

6. The process of alloy formation which comprises the steps of passing to a vaporizer a liquid phosphorous component and a liquid heat decomposable metal bearing compound to effect vaporization of the component and compound, combining the vapors of the component and compound, and contacting an object heated to the decomposition temperature of the combined vapors to effect the deposition of a phosphorous containing alloy on the object.

7. The process of alloy formation which comprises the steps of metering liquid trimethyl phosphine and liquid nickel carbonyl to a vaporizer to effect vaporization of the phosphine and carbonyl, combining the vapors of the carbonyl and phosphine in one atmosphere, and contacting an object heated to the decomposition temperature of the carbonyl and phosphine to effect deposition of a phosphorous-nickel alloy on the object.

8. The process of alloy formation which comprises the steps of metering liquid triethyl phosphine and liquid iron

pentacarbonyl to a vaporizer to effect vaporization of the phosphine and pentacarbonyl, combining the vapors of the carbonyl and phosphine in one atmosphere, and contacting an object heated to the decomposition temperature of the carbonyl and phosphine to effect deposition of a phosphorous-iron alloy on the object.

5 9. The process of alloy formation which comprises the steps of vaporizing tri-methyl phosphine and nickel carbonyl at a temperatures of between 112° F. and 170° F., 10 combining the vapors in a common atmosphere with an object heated to between 350° F. and 700° F. to thereby decompose the phosphine and carbonyl together to deposit an alloy of nickel-phosphorous on the object.

10 10. The process of alloy formation which comprises 15 the steps of vaporizing tri-ethyl phosphine and iron pentacarbonyl at a temperature of between 260° F. and 285° F., combining the vapors in a common atmosphere with an object heated to between 400° F. and 800° F. to thereby decompose the phosphine and pentacarbonyl together to deposit an alloy of iron-phosphorous on the object.

11 11. The process of alloy formation which comprises 20 the steps of vaporizing tri-methyl phosphine and nickel carbonyl, combining the vaporized phosphine and carbonyl in one atmosphere, providing an object heated to the decomposition tempertaure of the carbonyl and phosphine, and directing the combined phosphine and carbonyl atmosphere with a carrier gas into contact with the heated object to thereby effect deposition of a nickel-phosphorous alloy on the object.

#### References Cited in the file of this patent

##### UNITED STATES PATENTS

35 2,041,493 Schlecht et al. ----- May 19, 1936

##### FOREIGN PATENTS

376,652 Germany ----- June 4, 1923

##### OTHER REFERENCES

40 Zeitschrift für Anorganische Chemie, vol. 238 (1938),  
pages 72 and 73.